

## UNITED STATES PATENT OFFICE

2,155,728

## VAPOR PHASE BLEACHING

Paul La Frone Magill, Ransomville, N. Y., assignor to E. I. du Pont de Nemours & Company, Wilmington, Del., a corporation of Delaware

No Drawing. Application December 31, 1937,  
Serial No. 182,842

## 2 Claims. (Cl. 8—108)

This invention relates to a vapor phase process for the bleaching of various dark-colored materials which are now normally bleached in commercial operations. More particularly, it relates to the employment of the stable organic hypochlorite, tertiary butyl hypochlorite,



in the vapor phase for the bleaching of various materials.

The novel organic hypochlorite which I utilize for the vapor phase bleaching of materials, such as textile fabrics, fruits or other materials to be bleached, is a pale yellow mobile liquid having an irritating odor. It is exceedingly stable in the dark and may be kept for months if not exposed to the direct rays of sunlight. When exposed to direct sunlight it is but slightly decomposed but will quietly decompose upon prolonged exposure. It boils at a temperature of approximately 80° C. at atmospheric pressure and the vapors have been found to be exceedingly effective as a bleaching agent.

In a co-pending application of Paul J. Carlisle, Serial Number 182,625, filed December 30, 1937, the use of tertiary butyl hypochlorite as a bleaching and deodorizing agent for the treatment of textile fabrics, foodstuffs, oils, fats, waxes and other materials is disclosed. My invention relates solely to the use of this bleaching agent in the vapor phase, taking advantage of the fact that its boiling point at atmospheric pressure is approximately 80° C., and is not to be confused with the invention set forth in said co-pending application.

As an example of the use of tertiary butyl hypo-

chlorite for the vapor phase bleaching of various materials, the following may be given. It should be understood that this example is merely illustrative, and is not to be construed as restricting the nature of materials which I have succeeded in bleaching in the vapor phase by the use of vapors of tertiary butyl hypochlorite.

## Example

Tertiary butyl hypochlorite is vaporized at atmospheric pressure and the vapors carried by means of a current of air through dry cotton piece goods. At the end of fifteen minutes it was observed that the cotton was bleached to a substantial degree. After passage through the cotton the vapors were condensed, returned to the vaporizer, and again transmitted through the fabric. Similar results were obtained when treating other textile fabrics such as linen, wool, silk, etc.

It is to be understood that various changes might be made in the procedure described above which will still fall within the scope of my invention. The breadth of invention is to be determined, not by the details given merely as illustrative, but in accordance with the appended claims.

## I claim:

1. A process of bleaching dark-colored materials which comprises the step of contacting said materials with the vapors of tertiary butyl hypochlorite.

2. A process of bleaching a textile fabric which consists in passing vaporized tertiary butyl hypochlorite through said fabric.

PAUL LA FRONE MAGILL.

35